# EUROPEAN PATENT APPLICATION

(11) **EP 4 786 668 A1**
(43) Date of publication of application: **05.08.2026**
(21) Application number: 24871622.7
(22) Date of filing: 23.08.2024
(51) Int. Cl.: D04H 3/011, D04H 3/037, D04H 3/16

(54) **THREE-DIMENSIONAL NET-LIKE STRUCTURE**

(30) Priority: 28.09.2023 JP 2023168862
(71) Applicant: TOYOBO MC Corporation, Osaka-shi, Osaka 530-0001 (JP)
(72) Inventor: KAWANO, Fumika, Otsu-shi, Shiga 520-0292 (JP); TANIGUCHI, Keisuke, Otsu-shi, Shiga 520-0292 (JP); HENMI, Tatsuya, Otsu-shi, Shiga 520-0292 (JP)
(74) Representative: Müller-Boré & Partner Patentanwälte PartG mbB
(86) International application number: PCT/JP2024/029965
(87) International publication number: WO 2025/069820

(57) **Abstract**

It is provided that a biodegradable three-dimensional network structure that exhibits excellent compression recoverability after compression at a usage environment temperature and has excellent compression durabilities on both respective surfaces thereof, with the difference between the compression durabilities of both respective surfaces being small. A three-dimensional network structure having a three-dimensional random loop-bonded configuration and comprising a continuous filament made from a thermoplastic resin composition, wherein the thermoplastic resin composition contains 70% by mass or more of a polybutylene adipate terephthalate resin, an apparent density of one surface of the three-dimensional network structure is higher than an apparent density of the other surface of the three-dimensional network structure, a residual strain R₁ after compression is repeatedly performed 13,000 times at a load of 750 N from the one surface side and a residual strain R₂ after compression is repeatedly performed 13,000 times at a load of 750 N from the other surface side are each 20% or less, an absolute value of a difference between a value of the R₁ and a value of the R₂ is 10% or less, and the three-dimensional network structure has a 40°C-compression residual strain of 15% or less.

## Description

### TECHNICAL FIELD

The present invention relates to a three-dimensional network structure.

### BACKGROUND ART

To date, three-dimensional network structures are widely used as cushioning materials utilized for furniture, beddings such as beds, seats for vehicles such as electric trains, automobiles, and two-wheeled vehicles from the viewpoint of excellent air permeability and recyclability. Environment-related issues have been addressed in an accelerated manner recently. In view of this acceleration, research on biodegradable polymers that degrade in a shorter time than conventional polymers has been progressing for these three-dimensional network structures as well. Consequently, various technologies regarding biodegradable three-dimensional network structures have been disclosed to date.

Patent Document 1 discloses a technology of improving plant retaining properties of a biodegradable network structure. In addition, Patent Document 2 discloses a technology of improving local joining of a fiber material of a biodegradable network structure. In addition, Patent Document 3 discloses a technology of forming a coil spring-shaped or loop-shaped portion in a biodegradable three-dimensional structure so as to allow the portion to be suitably deformed under a compressive stress so that the stress is dispersed.

### CITATION LIST

### PATENT DOCUMENT

Patent Document 1: Japanese Laid-Open Patent Publication No. 2001-032236
Patent Document 2: Japanese Laid-Open Patent Publication No. 2020-128608
Patent Document 3: Japanese Laid-Open Patent Publication No. 2000-328422

### SUMMARY OF THE INVENTION

### PROBLEMS TO BE SOLVED BY THE INVENTION

In this manner, various attempts to improve the functions of biodegradable network structures have been made to date. However, there has yet to be a known biodegradable network body that exhibits both excellent cushioning properties and excellent recoverability at the time of compression at a usage environment temperature at which the biodegradable network body is used as a cushioning material. In particular, there has yet to be a known three-dimensional network structure having different cushioning performances on both respective surfaces thereof and having excellent compression durabilities on both respective surfaces thereof.

The present invention has been made in view of the above circumstances, and an object of the present invention is to provide a biodegradable three-dimensional network structure that exhibits excellent compression recoverability after compression at a usage environment temperature, the biodegradable three-dimensional network structure having excellent compression durabilities on both respective surfaces thereof, with the difference between the compression durabilities of both respective surfaces being small.

### SOLUTION TO THE PROBLEMS

That is, the present invention has the following invention.
[1] A three-dimensional network structure having a three-dimensional random loop-bonded configuration and comprising a continuous filament made from a thermoplastic resin composition, wherein the thermoplastic resin composition contains 70% by mass or more of a polybutylene adipate terephthalate resin, an apparent density of one surface of the three-dimensional network structure is higher than an apparent density of the other surface of the three-dimensional network structure, a residual strain R₁ after compression is repeatedly performed 13,000 times at a load of 750 N from the one surface side and a residual strain R₂ after compression is repeatedly performed 13,000 times at a load of 750 N from the other surface side are each 20% or less, an absolute value of a difference between a value of the R₁ and a value of the R₂ is 10% or less, and the three-dimensional network structure has a 40°C-compression residual strain of 15% or less.
[2] The three-dimensional network structure according to the above [1], wherein
   the polybutylene adipate terephthalate resin contains an adipic acid unit and a terephthalic acid unit, and a molar ratio of the terephthalic acid unit to the adipic acid unit is 1.0 or more and 3.0 or less.
[3] The three-dimensional network structure according to the above [1] or [2], wherein the polybutylene adipate terephthalate resin has a melting point of 125°C or more and 180°C or less.
[4] The three-dimensional network structure according to any one of the above [1] to [3], wherein the three-dimensional network structure has an apparent density of 0.005 g/cm³ or more and 0.20 g/cm³ or less.
[5] The three-dimensional network structure according to any one of the above [1] to [4], wherein, in a case where a larger value and a smaller value out of a 25%-compression hardness obtained upon pressure application from the one surface side and a 25%-compression hardness obtained upon pressure application from the other surface side are respectively defined as H₁ and H₂, H₁/H₂ is 1.03 or more.
[6] The three-dimensional network structure according to any one of the above [1] to [5], wherein, in a case where a larger value and a smaller value out of a 40%-compression hardness obtained upon pressure application from the one surface side and a 40%-compression hardness obtained upon pressure application from the other surface side are respectively defined as H₃ and H₄, H₃/H₄ is 1.05 or more.
[7] The three-dimensional network structure according to any one of the above [1] to [6], wherein an absolute value of a difference between a compressive deflection coefficient obtained upon pressure application from the one surface side and a compressive deflection coefficient obtained upon pressure application from the other surface side is 5.0 or less.
[8] The three-dimensional network structure according to any one of the above [1] to [7], wherein an enthalpy of an endothermic peak in which a differential scanning calorimetry curve regarding the continuous filament measured by using a differential scanning calorimeter has a minimum value in a range from 30°C to 70°C, is 2.5 J/g or less.
[9] The three-dimensional network structure according to any one of the above [1] to [8], wherein an absolute value of a difference between the apparent density of the one surface and the apparent density of the other surface is 0.015 g/cm³ or more.
[10] A cushioning material comprising the three-dimensional network structure according to any one of the above [1] to [9], wherein the cushioning material is reversibly usable.

### EFFECTS OF THE INVENTION

By employment of the above configuration, the three-dimensional network structure of the present invention exhibits excellent compression recoverability after compression at a usage environment temperature and has excellent compression durabilities on both respective surfaces thereof, with the difference between the compression durabilities of both respective surfaces being small.

### BRIEF DESCRIPTION OF THE DRAWING

[FIG. 1] FIG. 1 shows an example of a differential scanning calorimetry curve for measuring, in relation to a continuous filament forming a three-dimensional network structure, an enthalpy of an endothermic peak in which the differential scanning calorimetry curve has a minimum value in a range from 30°C to 70°C.

### DESCRIPTION OF EMBODIMENTS

The three-dimensional network structure of the present invention has a three-dimensional random loop-bonded configuration and comprises a continuous filament made from a thermoplastic resin composition. The thermoplastic resin composition contains 70% by mass or more of a polybutylene adipate terephthalate resin. In addition, an apparent density of one surface of the three-dimensional network structure is higher than an apparent density of the other surface of the three-dimensional network structure.

Employment of the above configuration enables the three-dimensional network structure to exhibit excellent compression recoverability after compression at a usage environment temperature and have excellent compression durabilities on both respective surfaces thereof, with the difference between the compression durabilities of both respective surfaces being small. The usage environment temperature means a temperature at which the three-dimensional network structure of the present invention is used as a product such as a cushion. In the present description, the usage environment temperature is defined as 40°C, and a 40°C-compression residual strain is used as an index of the compression recoverability after compression at the usage environment temperature. Hereinafter, the compression recoverability after compression at the usage environment temperature is sometimes simply referred to as "compression recoverability". Also, a post-repeated-compression residual strain is used as an index of each of the compression durabilities, and a smaller post-repeated-compression residual strain indicates a higher compression durability. Measurement methods for these indexes will be described later.

Hereinafter, each of the configurations will be described in detail.

### <Thermoplastic Resin Composition>

The thermoplastic resin composition forming the continuous filament contains 70% by mass or more of a polybutylene adipate terephthalate resin. By selecting the polybutylene adipate terephthalate resin from among biodegradable resins and using the thermoplastic resin composition containing 70% by mass or more of the polybutylene adipate terephthalate resin, a biodegradable three-dimensional network structure having excellent cushioning properties can be obtained. The polybutylene adipate terephthalate resin content is preferably 75% by mass or more, more preferably 80% by mass or more, further preferably 90% by mass or more, particularly preferably 95% by mass or more, and most preferably 99% by mass or more with respect to the amount of the thermoplastic resin composition. The thermoplastic resin composition forming the continuous filament may contain 100% by mass of the polybutylene adipate terephthalate resin.

The polybutylene adipate terephthalate resin is a biodegradable thermoplastic resin and is a copolymer of adipic acid, terephthalic acid, and butanediol. By having biodegradability, the polybutylene adipate terephthalate resin is expected to become one solution to problems arising from disposal of rubbish and problems regarding microplastics. The adipic acid, the terephthalic acid, and the butanediol do not need to be simultaneously copolymerized and may be copolymerized in multiple stages.

In the polybutylene adipate terephthalate resin, a molar ratio of the terephthalic acid unit to the adipic acid unit is preferably 1.0 or more and 3.0 or less, more preferably 1.1 or more and 2.5 or less, further preferably 1.2 or more and 2.0 or less, and even more preferably 1.3 or more and 1.8 or less. By the molar ratio being 1.0 or more, the compression durabilities of both respective surfaces of the three-dimensional network structure, and the compression recoverability after compression at the usage environment temperature of the three-dimensional network structure, are easily improved. Meanwhile, by the molar ratio being 3.0 or less, flexibility is improved, and the difference between the compression durabilities of both respective surfaces becomes small. Therefore, the three-dimensional network structure becomes suitable as a cushioning material or the like.

The polybutylene adipate terephthalate resin has a melting point of preferably 125°C or more and 180°C or less, more preferably 130°C or more and 175°C or less, further preferably 135°C or more and 170°C or less, particularly preferably 140°C or more and 165°C or less, and most preferably 145°C or more and 160°C or less. By the melting point being 125°C or more, the compression recoverability after compression at the usage environment temperature of the three-dimensional network structure can be easily improved. Meanwhile, by the melting point being 180°C or less, the three-dimensional network structure exhibits an improved flexibility and can be suitably used as a cushioning material or the like.

The polybutylene adipate terephthalate resin has a melt flow rate (MFR) of preferably 3 g/10 min to 60 g/10 min. When the MFR is 3 g/10 min or more, the compression recoverability and the compression durabilities of both respective surfaces are easily increased. Meanwhile, when the MFR is 60 g/10 min or less, the melt viscosity can be increased, and the fiber diameter of the continuous filament can be increased. The MFR is more preferably 4 g/10 min to 50 g/10 min, further preferably 5 g/10 min to 40 g/10 min, particularly preferably 6 g/10 min to 18 g/10 min, and most preferably 10 g/10 min to 15 g/10 min. The MFR of the thermoplastic resin composition forming the continuous filament is also preferably within this range. The MFR of the resin can be measured through a method explained in EXAMPLES described later.

When using a commercially available resin as a polybutylene adipate terephthalate resin, in case where a resin has a low melt flow rate (MFR), MFR of the resin can be increased by adding water to the resin to cause hydrolysis of the resin during melt extrusion. Meanwhile, in case where a resin has a high MFR, MFR of the resin can be reduced by drying the resin and then melt extruding.

The thermoplastic resin composition forming the continuous filament may include another biodegradable resin other than polybutylene adipate terephthalate resin. The biodegradable resin other than polybutylene adipate terephthalate resin preferably include polylactic acid, polylactic acid/polycaprolactone copolymer, polylactic acid/polyether copolymer, polyethylene terephthalate succinate, polybutylene succinate, polybutylene succinate adipate, polyglycolic acid, polycaprolactone, polyvinyl alcohol, cellulose acetate, and the like. These resins may be used alone or in combination. Details of the resins are shown in the positive list of green plastic (biodegradable plastic) with a classification number A-1 published by Japan BioPlastics Association. The thermoplastic resin composition forming the continuous filament may include a resin other than biodegradable resin. Examples of the resin include thermoplastic resins such as polyolefin, polyurethane, and polyester.

In addition, the thermoplastic resin composition forming the continuous filament may contain not only the polybutylene adipate terephthalate resin but also a resin having other copolymerization components other than adipic acid, terephthalic acid, and butanediol as units. Examples of the other copolymerization component include any dicarboxylic acid other than adipic acid and terephthalic acid, any diol other than butanediol, polyalkylene glycol, and a modifier for chain extension or end capping. These may be used alone or in combination.

Examples of the dicarboxylic acid other than adipic acid and terephthalic acid include oxalic acid, malonic acid, succinic acid, glutaric acid, pimelic acid, and suberic acid. These may be used alone or in combination.

Examples of the diol other than butanediol include methanediol, ethanediol, propanediol, pentanediol, and hexanediol. Example of the polyalkylene glycol include polymethylene glycol, polyethylene glycol, polypropylene glycol, and polybutylene glycol (polytetramethylene glycol). These may be used alone or in combination.

The modifier may be, for example, a polyisocyanate compound or a glycol compound. The polyisocyanate compound may be, for example, a diisocyanate compound.

Examples of the diisocyanate compound include hexamethylene diisocyanate, 4,4'-diphenylmethane diisocyanate, 2,4-tolylene diisocyanate, 2,6-tolylene diisocyanate, xylylene diisocyanate, 1,5-naphthylene diisocyanate, p-phenylene diisocyanate, isophorone diisocyanate, 4,4'-dicyclohexylmethane diisocyanate, tetra-methyl xylene diisocyanate, carbodiimide modified MDI, and polymethylene phenyl polyisocyanate. These compounds may be used alone or in combination.

As a monomer for synthesizing the thermoplastic resin composition forming the continuous filament, a petroleum-derived monomer may be used. However, biomass-derived monomers are preferable from the viewpoint of lowering environmental load. As to the biomass-derived monomers, for example, monomers shown in a positive list with a classification number A (biomass-derived plastic) published by Japan BioPlastics Association can be used.

The total amount of the adipic acid unit and the terephthalic acid unit contained per 100 mol% of the dicarbon units contained in the thermoplastic resin composition forming the continuous filament is preferably 70 mol% or more, more preferably 80 mol% or more, further preferably 90 mol% or more, even more preferably 95 mol% or more, and particularly preferably 99 mol% or more. The amount of the butanediol unit contained per 100 mol% of the diol units contained in the thermoplastic resin composition forming the continuous filament is preferably 70 mol% or more, more preferably 80 mol% or more, further preferably 90 mol% or more, even more preferably 95 mol% or more, and particularly preferably 99 mol% or more.

In order to impart desired functions, the thermoplastic resin composition forming the continuous filament may contain additives. Examples of the additives include a deodorant agent, an antibacterial agent, an antifungal agent, an anti-mite agent, an anti-odor agent, an antimycotic agent, an aromatic agent, a flame retardant, a moisture absorbing/releasing agent, an antioxidant, and a lubricant. These may be used alone or in combination.

Examples of the antioxidant include known phenol-based antioxidant, phosphite-based antioxidant, thioether-based antioxidant, benzotriazole-based UV absorber, triazine-based UV absorber, benzophenone-based UV absorber, N-H type hindered amine-based light stabilizer, and N-CH₃ type hindered amine-based light stabilizer.

Examples of the phenol-based antioxidant include 1,3,5-tris[[3,5-bis(1,1-dimethylethyl)-4-hydroxyphenyl]methyl]-1,3,5-triazine-2,4,6(1H,3H,5H)-trione, 1,1,3-tris(2-methyl-4-hydroxy-5-tert-butylphenyl)butane, 4,4'-butylidenebis(6-tert-butyl-m-cresol), 3-(3,5-di-tert-butyl-4-hydroxyphenyl)propionic acid stearyl, pentaerythritol tetrakis[3-(3,5-di-tert-butyl-4-hydroxyphenyl)propionate], 2,2'-dimethyl-2,2'-(2,4,8,10-tetraoxaspiro[5.5]undecane-3,9-diyl)dipropane-1,1'-diyl bis[3-(3-tert-butyl-4-hydroxy-5-methylphenyl)propanoate] and 2,4,6-tris(3',5'-di-tert-butyl-4'-hydroxybenzyl)mesitylene.

Examples of the phosphite-based antioxidant include 3,9-bis(octadecyloxy)-2,4,8,10-tetraoxa-3,9-diphosphaspiro[5,5]undecane, 3,9-bis(2,6-di-tert-butyl-4-methylphenoxy)-2,4,8,10-tetraoxa-3,9-diphosphaspiro[5,5]undecane, 2,4,8,10-tetrakis(1,1-dimethylethyl)-6-[(2-ethylhexyl)oxy]-12H-dibenzo[d,g][1,3,2]dioxaphosphocin, tris(2,4-di-tert-butylphenyl)phosphite, tris(4-nonylphenyl)phosphite, tetraalkyl(C12-15)-4,4'-isopropylidenediphenyl diphosphite, diphenyl(2-ethylhexyl)phosphite, diphenyl isodecyl phosphite, triisodecyl phosphite, and triphenyl phosphite.

Examples of the thioether-based antioxidant include bis[3-(dodecylthio)propionate]2,2-bis[[3-(dodecylthio)-1-oxopropyloxy]methyl]-1,3-propanediyl and 3,3'-ditridecyl thiobispropionate.

In order to prevent thermal degradation of the thermoplastic resin, a mixture of phenol-based antioxidant and a phosphite-based antioxidant may be used.

Examples of the lubricant include hydrocarbon-based waxes, higher alcohol-based waxes, amide-based waxes, ester-based waxes, and metal soap.

### <Continuous Filament>

The three-dimensional network structure of the present invention has a three-dimensional random loop-bonded configuration and is made of a continuous filament made from the thermoplastic resin composition. The continuous filament is a linear filament having a continuous portion of at least 5 mm or more. Presence of a portion obtained by adhering intersections of such continuous filaments makes it easy to form a three-dimensional network structure. Therefore, the three-dimensional network structure preferably has an adhesion portion at which the intersections of the continuous filaments have been adhered to each other.

If a hollow fiber and a solid fiber have equal finenesses, the hollow fiber has a higher second moment of area than the solid fiber. Thus, use of the hollow fiber for the continuous filament forming the three-dimensional network structure of the present invention leads to a higher resistance to compression than use of the solid fiber for this continuous filament. Therefore, both the hollow fiber and the solid fiber are preferably used in order to obtain different cushioning performances on both respective surfaces. The hollow fiber means a fiber having a hollow cross section, and the solid fiber means a fiber having a solid cross section.

The hollow fiber has a degree of hollowness of preferably 1 to 30%, more preferably 2 to 30%, and particularly preferably 5 to 25% or more. The degree of hollowness can be measured through a method explained in EXAMPLES described later. Meanwhile, the solid fiber has a degree of hollowness of less than 1%.

In addition, an average fiber diameter of such hollow fibers is preferably larger than an average fiber diameter of such solid fibers in order to obtain different cushioning performances on both respective surfaces. In a case where the average fiber diameter of the hollow fibers is larger than the average fiber diameter of the solid fibers, the difference between the average fiber diameter of the hollow fibers and the average fiber diameter of the solid fibers is preferably 0.12 to 2.5 mm, more preferably 0.14 to 1.0 mm, further preferably 0.16 to 0.40 mm, and particularly preferably 0.20 to 0.35 mm. When the difference between the average fiber diameter of the hollow fibers and the average fiber diameter of the solid fibers is 0.12 mm or more, the three-dimensional network structure is easily caused to have different cushioning performances on both respective surfaces thereof.

The average fiber diameter of the hollow fibers is preferably 0.1 mm or more and 3.0 mm or less, more preferably 0.3 mm or more and 2.0 mm or less, further preferably 0.5 mm or more and 1.5 mm or less, and even more preferably 0.6 mm or more and 1.0 mm or less. The average fiber diameter of the solid fibers is preferably 0.1 mm or more and 3.0 mm or less, more preferably 0.2 mm or more and 2.0 mm or less, further preferably 0.3 mm or more and 1.5 mm or less, and even more preferably 0.4 mm or more and less than 0.6 mm.

Although each of the solid fibers and the hollow fibers preferably has a substantially circular shape, there is also a case where causing each of the fibers to have an atypical cross section makes it possible to impart resistance to compression and touch characteristics. Also, the continuous filament forming the three-dimensional network structure of the present invention may be a composite filament obtained by combination with a continuous filament made from another thermoplastic resin as long as the object of the present invention is achieved. Examples of the type of such a composite in the case of compositing the filament itself include a sheath-core type, a side-by-side type, an eccentric sheath-core type, and the like.

The continuous filament preferably has an enthalpy of fusion of 16 to 30 J/g. By the enthalpy of fusion being 16 J/g or more, the compression durabilities and the compression recoverability of the three-dimensional network structure can be improved. Meanwhile, by the enthalpy of fusion being 30 J/g or less, the flexibility of the three-dimensional network structure can be improved, whereby noise that might be generated during compression and during recovery can be decreased. The enthalpy of fusion is more preferably 17 J/g or more, further preferably 18 J/g or more, even more preferably 19 J/g or more, still even more preferably 20 J/g or more, and particularly preferably 21 J/g or more. Meanwhile, the enthalpy of fusion is more preferably 28 J/g or less.

An enthalpy (J/g) of an endothermic peak of the continuous filament can be obtained from an integral value of an endothermic peak (melting peak) based on a DSC curve measured under a nitrogen atmosphere and at a heating rate of 20°C/min by using a differential scanning calorimeter, with a sample mass being set to 2.0 mg±0.1 mg. The integral value can be obtained as follows. That is, a point at which the curve related to the aforementioned endothermic peak (melting peak) starts to be away from a baseline on the low-temperature side is defined as a start point, a point at which the curve starts to be in contact with a baseline on the high-temperature side is defined as an end point, a straight line connecting the start point and the end point is drawn, and integration is performed on the portion enclosed by the straight line and the curve. An example of the DSC curve is shown in FIG. 1. A broken line in FIG. 1 is the straight line connecting the above start point and the above end point of the endothermic peak (melting peak), and the portion enclosed by the broken line and the curve is an integration region on which integration is performed.

The enthalpy of the endothermic peak in which the DSC curve regarding the continuous filament forming the three-dimensional network structure measured by using a differential scanning calorimeter has a minimum value in a range from 30°C to 70°C, is preferably 2.5 J/g or less. The "enthalpy of the endothermic peak in which the DSC curve has a minimum value in the range from 30°C to 70°C" is sometimes expressed as a low-temperature phase enthalpy in the present invention. By the low-temperature phase enthalpy being 2.5 J/g or less, the 40°C-compression residual strain is easily decreased. As a result, feeling of irrecoverable deformation when the three-dimensional network structure is used as a cushioning material is easily decreased. Considering this advantage, the low-temperature phase enthalpy is more preferably 1.5 J/g or less. The lower limit of the low-temperature phase enthalpy is not particularly limited, but the low-temperature phase enthalpy is, for example, 0.2 J/g or more in consideration of technical difficulties.

### <Configuration of Three-Dimensional Network Structure>

Before a configuration of the three-dimensional network structure of the present invention is explained, a typical network structure including a hollow fiber and a solid fiber will be described first.

For example, a laminated network structure in which a network structure made of the hollow fiber and a network structure made of the solid fiber have been stacked is formed, whereby different cushioning performances can be imparted on both respective surfaces thereof. Although such a laminated network structure enables different cushioning performances to be imparted on both respective surfaces, the above laminated network structure has the following drawback. That is, when compression is performed by pressure application from a surface of a network structure having a lower compression hardness out of the network structures, only the network structure having the lower compression hardness is deformed by the compression first, and only the network structure having the lower compression hardness is warped independently of a network structure having a higher compression hardness out of the network structures. Then, when the network structure having the lower compression hardness becomes unable to withstand the compression load alone, the compressive stress finally propagates to the network structure having the higher compression hardness, and the network structure having the higher compression hardness starts to be deformed or warped. Thus, if such compression is repeated, fatigue is accumulated in the network structure having the lower compression hardness, and the network structure having the lower compression hardness comes to have a decreased thickness or a decreased compression hardness. That is, in the above laminated network structure, although different cushioning performances can be imparted on both respective surfaces, repeated application of pressure leads to increase in residual strain of the network structure having the lower compression hardness, whereby the difference between the compression durabilities of both respective surfaces of the laminated network structure becomes significantly large.

It is conceivable to obtain, as a laminated network structure other than the above laminated network structure, a laminated network structure in which the network structure made of the hollow fiber and the network structure made of the solid fiber have been integrated by being adhered to each other by using an adhesive. Such a laminated network structure enables different cushioning performances to be imparted on both respective surfaces thereof. However, although both network structures are integrally deformed and warped upon a compression load by pressure application while the number of times of compression is small, further repetition of compression leads to further concentration of stress on the adhesion surfaces. Consequently, the adhesive force therebetween is weakened, or peeling occurs. Thus, in the laminated network structure in which the structures have been adhered to each other as well, the difference between the compression durabilities of both respective surfaces becomes significantly large.

It is also possible to obtain a laminated network structure in which: the solid fiber is extruded onto the network structure made of the hollow fiber so that the network structure made of the solid fiber is stacked; and these network structures are integrated by being fused to each other so that the laminated network structure has a three-dimensional network configuration. Such a laminated network structure enables different cushioning performances to be imparted on both respective surfaces thereof. However, since the solid fiber is fused after the hollow fiber is solidified once, fusion force between the boundary surfaces of the hollow fiber layer and the solid fiber layer is weak, and repeated reception of a compression load leads to concentration of stress on the boundary surfaces, whereby interfacial peeling occurs. As a result, durability deteriorates.

The present inventors have found that presence of a coexistence region in which the solid fiber and the hollow fiber coexist between a region present on one surface side and mainly composed of the hollow fiber and a region present on the other surface side and mainly composed of the solid fiber (hereinafter, simply referred to as "coexistence region") enables decrease in the difference between post-repeated-compression residual strains of both respective surfaces (enables decrease in the difference between the compression durabilities of both respective surfaces).

In each of the three laminated network structures described above, such a coexistence region is not present at all or is hardly present. However, when a three-dimensional network structure in which the region mainly composed of the hollow fiber, the coexistence region, and the region mainly composed of the solid fiber have been stacked in this order from the one surface side toward the other surface side is formed, since the coexistence region is present in a region located near the midpoint between both surfaces, a three-dimensional network structure in which the region mainly composed of the hollow fiber, the coexistence region, and the region mainly composed of the solid fiber are integrated without being separated from each other is formed. Therefore, even when compression is performed by pressure application from the low-compression-hardness side, stress propagates through the coexistence region to the high-compression-hardness side upon compression by pressure application while the number of times of compression is still small. Thus, the stress is efficiently dispersed in the thickness direction, whereby the entire network structure is deformed and warped upon the compression load by pressure application. Consequently, the difference between compression durability obtained upon pressure application from the low-compression-hardness side and compression durability obtained upon pressure application from the high-compression-hardness side can be made small. In the case of the three-dimensional network structure in which the region mainly composed of the hollow fiber, the coexistence region, and the region mainly composed of the solid fiber have been stacked in this order, it is preferable that the region mainly composed of the hollow fiber and the region mainly composed of the solid fiber are respectively present on one surface (high-density surface) and the other surface (low-density surface) from the viewpoint of causing the one surface to have a higher apparent density than the other surface.

### <Physical Properties of Three-Dimensional Network Structure>

The three-dimensional network structure of the present invention is characterized in that: both a post-repeated-compression residual strain obtained upon pressure application from the one surface (high-density surface) side and a post-repeated-compression residual strain obtained upon pressure application from the other surface (low-density surface) side are low; and both surfaces have excellent compression durabilities. Specifically, a residual strain R₁ after compression is repeatedly performed 13,000 times at a load of 750 N from the one surface (high-density surface) side and a residual strain R₂ after compression is repeatedly performed 13,000 times at a load of 750 N from the other surface (low-density surface) side are each 20% or less. Both R₁ and R₂ are preferably 15% or less, more preferably 13% or less, further preferably 10.5% or less, and particularly preferably 9.5% or less.

The three-dimensional network structure of the present invention is characterized also in that the difference between the compression durabilities of both respective surfaces thereof, i.e. the difference between the post-repeated-compression residual strain obtained upon pressure application from the one surface (high-density surface) side and the post-repeated-compression residual strain obtained upon pressure application from the other surface (low-density surface) side, is small. Specifically, the absolute value of the difference between the value of the R₁ and the value of the R₂ is 10% or less. When the absolute value of the difference between the value of the R₁ and the value of the R₂ exceeds 10%, the difference between the post-repeated-compression residual strains of both respective surfaces becomes excessively large. Consequently, when the three-dimensional network structure of the present invention is reversibly used, the extent of feeling of irrecoverable deformation of the surface on the side on which the post-repeated-compression residual strain has a large value becomes larger than the extent of feeling of irrecoverable deformation of the surface on the side on which the post-repeated-compression residual strain has a small value. The absolute value of the difference between the value of the R₁ and the value of the R₂ is preferably 9% or less, more preferably 8% or less, further preferably 6% or less, and particularly preferably 1.5% or less. The lower limit of the absolute value of the difference between the value of the R₁ and the value of the R₂ is not particularly limited, and the absolute value is, for example, 0% or more and preferably 0.1% or more.

The three-dimensional network structure has a 40°C-compression residual strain of 15% or less and preferably 14.5% or less. By setting the 40°C-compression residual strain to be 15% or less, the compression recoverability can be improved. The lower limit of the 40°C-compression residual strain is not limited, and the 40°C-compression residual strain is, for example, 1% or more and preferably 5% or more. The 40°C-compression residual strain can be measured through a method explained in EXAMPLES described later.

In a case where pressure is applied to the three-dimensional network structure from the high-density surface thereof, a compression hardness obtained upon compression by 25% in the thickness direction (upon compression to a 75% thickness) (hereinafter, referred to as "25%-compression hardness") is preferably 5.0 N/φ50 mm or more and 100 N/φ50 mm or less, more preferably 8.0 N/φ50 mm or more and 80.0 N/φ50 mm or less, further preferably 10.0 N/φ50 mm or more and 50.0 N/φ50 mm or less, particularly preferably 12.0 N/φ50 mm or more and 30.0 N/φ50 mm or less, and most preferably 15.0 N/φ50 mm or more and 25.0 N/φ50 mm or less. By the 25%-compression hardness being 5.0 N/φ50 mm or more, bottom-touch feeling when the three-dimensional network structure is used as a cushioning material or the like can be decreased. Meanwhile, by the 25%-compression hardness being 100 N/φ50 mm or less, cushioning properties can be improved. The 25%-compression hardness can be measured through a method explained in EXAMPLES described later.

In a case where pressure is applied to the three-dimensional network structure from the low-density surface thereof, the 25%-compression hardness is preferably 5.0 N/φ50 mm or more and 100 N/φ50 mm or less, more preferably 5.0 N/φ50 mm or more and 80.0 N/φ50 mm or less, further preferably 8.0 N/φ50 mm or more and 50.0 N/φ50 mm or less, particularly preferably 10.0 N/φ50 mm or more and 25.0 N/φ50 mm or less, and most preferably 12.0 N/φ50 mm or more and 20.0 N/φ50 mm or less. By the 25%-compression hardness being 5.0 N/φ50 mm or more, bottom-touch feeling when the three-dimensional network structure is used as a cushioning material or the like can be decreased. Meanwhile, by the 25%-compression hardness being 100 N/φ50 mm or less, cushioning properties can be improved.

In a case where a larger value and a smaller value out of the 25%-compression hardness obtained upon pressure application from the high-density surface side and the 25%-compression hardness obtained upon pressure application from the low-density surface side are respectively defined as H₁ and H₂, H₁/H₂ is preferably 1.03 or more, more preferably 1.05 or more, further preferably 1.07 or more, particularly preferably 1.10 or more, and most preferably 1.13 or more. In a case where the ratio between the 25%-compression hardnesses is less than 1.03, the difference between the cushioning performances of both respective surfaces might become small. The upper limit of H₁/H₂ is not particularly limited, and H₁/H₂ is, for example, 1.50 or less and preferably 1.40 or less.

In the case where pressure is applied to the three-dimensional network structure from the high-density surface thereof, a compression hardness obtained upon compression by 40% in the thickness direction (upon compression to a 60% thickness) (hereinafter, referred to as "40%-compression hardness") is preferably 10 N/φ50 mm or more and 500 N/φ50 mm or less, more preferably 15 N/φ50 mm or more and 300 N/φ50 mm or less, further preferably 17 N/φ50 mm or more and 200 N/φ50 mm or less, particularly preferably 20 N/φ50 mm or more and 100 N/φ50 mm or less, and most preferably 22 N/φ50 mm or more and 50 N/φ50 mm or less. By the 40%-compression hardness being 10 N/φ50 mm or more, bottom-touch feeling when the three-dimensional network structure is used as a cushioning material or the like can be decreased. Meanwhile, by the 40%-compression hardness being 500 N/φ50 mm or less, cushioning properties can be improved. The 40%-compression hardness can be measured through a method explained in EXAMPLES described later.

In the case where pressure is applied to the three-dimensional network structure from the low-density surface thereof, the 40%-compression hardness is preferably 10 N/φ50 mm or more and 500 N/φ50 mm or less, more preferably 12 N/φ50 mm or more and 300 N/φ50 mm or less, further preferably 15 N/φ50 mm or more and 200 N/φ50 mm or less, particularly preferably 17 N/φ50 mm or more and 100 N/φ50 mm or less, and most preferably 20 N/φ50 mm or more and 40 N/φ50 mm or less. By the 40%-compression hardness being 10 N/φ50 mm or more, bottom-touch feeling when the three-dimensional network structure is used as a cushioning material or the like can be decreased. Meanwhile, by the 40%-compression hardness being 500 N/φ50 mm or less, cushioning properties can be improved.

In a case where a larger value and a smaller value out of the 40%-compression hardness obtained upon pressure application from the high-density surface side and the 40%-compression hardness obtained upon pressure application from the low-density surface side are respectively defined as H₃ and H₄, H₃/H₄ is preferably 1.05 or more, more preferably 1.07 or more, and further preferably 1.09 or more. In a case where the ratio between the 40%-compression hardnesses is less than 1.05, the difference between the cushioning performances of both respective surfaces might become small. The upper limit of H₃/H₄ is not particularly limited, and H₃/H₄ is, for example, 1.50 or less and preferably 1.40 or less.

Both a compressive deflection coefficient obtained upon pressure application from the high-density surface side and a compressive deflection coefficient obtained upon pressure application from the low-density surface side are preferably 2.5 or more and 10.0 or less. When either of the compressive deflection coefficients is less than 2.5, the difference between the cushioning performances relative to change in a compression rate is small, and comfort in sleeping or comfort in sitting might deteriorate. In contrast, when either of the compressive deflection coefficients exceeds 10.0, the difference between the cushioning performances becomes excessively large according to change in the compression rate, whereby bottom-touch feeling or feeling of awkwardness might be perceived.

The compressive deflection coefficient obtained upon pressure application from the high-density surface is more preferably 2.6 or more and 8.0 or less, further preferably 2.7 or more and 6.0 or less, and particularly preferably 2.7 or more and 5.0 or less. The compressive deflection coefficient obtained upon pressure application from the low-density surface is more preferably 2.8 or more and 8.0 or less, further preferably 3.0 or more and 7.0 or less, and particularly preferably 3.5 or more and 6.0 or less.

The absolute value of the difference between the compressive deflection coefficient obtained upon pressure application from the high-density surface side and the compressive deflection coefficient obtained upon pressure application from the low-density surface side is preferably 5.0 or less, more preferably 3.0 or less, further preferably 2.0 or less, particularly preferably 1.5 or less, and most preferably 1.2 or less. When the absolute value of the difference between the compressive deflection coefficients exceeds 5.0, bottom-touch feeling or feeling of awkwardness might be perceived during use of the surface having the higher compressive deflection coefficient. The lower limit of the absolute value of the difference between the compressive deflection coefficients is not particularly limited, and the absolute value is, for example, 0 or more and preferably 0.1 or more. The compressive deflection coefficient obtained upon pressure application from the low-density surface side is preferably larger than the compressive deflection coefficient obtained upon pressure application from the high-density surface side.

The three-dimensional network structure has an apparent density of preferably 0.005 g/cm³ to 0.20 g/cm³, more preferably 0.010 g/cm³ to 0.17 g/cm³, further preferably 0.020 g/cm³ to 0.15 g/cm³, particularly preferably 0.030 g/cm³ to 0.12 g/cm³, and most preferably 0.045 g/cm³ to 0.10 g/cm³. By the apparent density being 0.005 g/cm³ or more, the hardness of the three-dimensional network structure is improved. As a result, bottom-touch feeling when the three-dimensional network structure is used as a cushioning material or the like can be decreased. Meanwhile, by the apparent density being 0.30 g/cm³ or less, the three-dimensional network structure exhibits an improved flexibility and can be suitably used as a cushioning material or the like. The apparent density of the three-dimensional network structure can be measured through a method explained in EXAMPLES described later.

Since the three-dimensional network structure of the present invention has different cushioning performances on both respective surfaces thereof, an apparent density of one of the surfaces is higher than an apparent density of the other one of the surfaces. The absolute value of the difference between the apparent density of the one surface (high-density surface) and the apparent density of the other surface (low-density surface) is preferably 0.015 g/cm³ or more, more preferably 0.020 to 0.100 g/cm³, and further preferably 0.030 to 0.080 g/cm³. The apparent densities of the one surface and the other surface of the three-dimensional network structure can be measured through a method explained in EXAMPLES described later.

The three-dimensional network structure has a thickness of preferably 10 mm to 120 mm. By the thickness being 10 mm or more, the three-dimensional network structure is easily used as a cushioning material or the like. Considering this, regarding the lower limit of this thickness, the thickness is more preferably 15 mm or more, further preferably 20 mm or more, and particularly preferably 22 mm or more. Meanwhile, regarding the upper limit of this thickness, the thickness is more preferably 100 mm or less, further preferably 80 mm or less, and particularly preferably 50 mm or less in consideration of the size of a manufacturing apparatus. The thickness of the three-dimensional network structure can be measured through a method explained in EXAMPLES described later.

The three-dimensional network structure is preferably free from a bonding promoter. The absence of a bonding promoter prevents excessive hardening generated by excessive bonding due to bonding promoter in the three-dimensional network structure. In addition, a decrease in fineness of the three-dimensional network structure caused by excessively increased bonding area per one contact point may be prevented. Examples of the bonding promoter include polycaprolactone, polybutylene succinate, polybutylene sebacate terephthalate, and polybutylene azelate terephthalate.

The three-dimensional network structure may be colored. A color agent such as a pigment or a dye can be used. The color agent may be contained in the resin before melt spinning, or the continuous filaments may be coated with a color agent by immersion or application after the formation of the three-dimensional network structure.

The shape of the three-dimensional network structure is not particularly limited. Examples of the shape of the three-dimensional network structure include a plate, triangular, quadrangular such as polygonal, cylindrical, spherical shape, or combinations thereof. The three-dimensional network structure may be obtained by molding with baffles when resin is melt extruded, or may be molded by a method such as cutting or hot pressing.

A reversibly usable cushioning material including the above specified three-dimensional network structure is also encompassed in the present invention. Being reversibly usable means being usable as a cushion at each of the high-density surface and the low-density surface, but the cushioning material of the present invention encompasses a case of being used as a cushioning material at only one of the surfaces.

Examples of the cushion include cushions for office chairs, furniture, sofas, bedding such as beds, cushions for seats of vehicles such as trains, automobiles, two-wheeled vehicles, child safety seats, and baby buggies, shock-absorbing mats such as floor mats and members for preventing collision and nipping.

### <Manufacturing Method for Three-dimensional Network Structure>

Hereinafter, the manufacturing method of the three-dimensional network structure in which the region mainly composed of the hollow fiber, the coexistence region, and the region mainly composed of the solid fiber have been stacked in this order from the one surface side toward the other surface side will be described.

The manufacturing method for the three-dimensional network structure preferably includes: an extrusion step of extruding, from a nozzle, the thermoplastic resin composition melted; a molding step of molding the continuous filament made from the thermoplastic resin composition extruded from the nozzle, into a three-dimensional network configuration so as to obtain a molded body; and a heat treatment step of heat treating the molded body. A three-dimensional network structure for which the heat treatment step has not been finished is referred to as a molded body in order to avoid confusion with a three-dimensional network structure as a finished product (a three-dimensional network structure for which the heat treatment step has been finished). The extrusion step and the molding step are not particularly limited as long as these steps are performed through a publicly known manufacturing method. Specific examples of the manufacturing method include the following method.

First, the thermoplastic resin composition including polybutylene adipate terephthalate resin is distributed to nozzle orifices of a multi-row nozzle having a plurality of orifices having a plurality of different orifice hole diameters, and then discharged downward from the nozzle at a spinning temperature, which is melting point of the resin +20°C or higher and lower than melting point of the resin +180°C. Specific examples of the multi-row nozzle will be described later. Next, a three-dimensional network configuration is formed by bringing continuous filaments into contact with each other in a melt state and fusing contact portions thereof, then the configuration is sandwiched with take-up conveyor nets, and cooled with a cooling water in a water tank. After cooling, the solidified molded body is drawn, then drained or dried, and the molded body having two or one smoothed side can be obtained. With regard to the spinning process and the cooling process, for example, descriptions in Japanese Laid-Open Patent Publication No. H7-68061 can be referenced. In case where only one surface needs to be smoothed, continuous filaments are discharged on an inclined take-up net, and the continuous filaments are contacted with each other and fused at contact portions thereof in a melt state. While the three-dimensional network configuration is being formed, the shape only on the take-up net touching side of the configuration may be loosened and the configuration may be cooled. The obtained molded body may be subjected to a heat treatment. The drying treatment of the molded body may be the heat treatment.

As a means of adjusting flexibility, water may be added to the thermoplastic resin composition before the resin is discharged from a nozzle. Water is added preferably at 2.0% by mass or less with respect to the thermoplastic resin composition.

Water may be added to the thermoplastic resin composition in any manner. For example, the thermoplastic resin composition may be absolutely dried in vacuum at 100°C for 12 hours or more before discharged from a nozzle, and a predetermined amount of water may be added with respect to 100% by mass of absolutely dried thermoplastic resin composition.

After melt-molding, the polybutylene adipate terephthalate resin is cooled preferably with cooling water. The polybutylene adipate terephthalate resin may shrink in molding by the time the resin is solidified by cooling. Because of the molding shrinkage phenomenon, the three-dimensional network structure should preferably be formed to have a width and a thickness in consideration of molding shrinkage. For example, by lowering the solidification temperature of melting resin, the shrinkage in molding can be reduced. Therefore, the temperature of the cooling water in the water tank is preferably 20°C or lower, and more preferably 15°C or lower. The resin is preferably cooled with cooling water with the cooling time of preferably 30 seconds or more. The resin is preferably solidified by cooling in a water tank.

The heat treatment may be conducted in a commercially available hot-air drying oven or may be in a warm water bath. The heat treatment temperature is preferably 50°C or higher. The heat treatment under such conditions can increase an enthalpy of fusion. The heat treatment temperature is more preferably 60°C or higher, and further preferably 70°C or higher. The heat treatment may be performed multiple times at different temperatures.

For performing the heat treatment, the thermoplastic resin composition forming the continuous filament preferably has a melting point of 125°C or higher and 180°C or lower. The lower limit of the melting point is more preferably 130°C or higher, further preferably 135°C or higher, even more preferably 140°C or higher, and particularly preferably 145°C or higher. Meanwhile, the upper limit of the melting point is more preferably 170°C or lower and further preferably 160°C or lower. When the melting point is 125°C or higher, the heat treatment can be performed in a suitable temperature range. Meanwhile, when the melting point is 180°C or lower, the three-dimensional network structure exhibits an improved flexibility, and thus, can be suitably used as a cushioning material or the like.

The heat treatment time in each heat treatment step is preferably 1 minute or more. This can increase an enthalpy of fusion. The heat treatment time is more preferably 5 minutes or more, further preferably 10 minutes or more, and particularly preferably 15 minutes or more. Meanwhile, the upper limit of the heat treatment time in each heat treatment step is preferably 60 minutes or less, and more preferably 50 minutes or less. This can reduce yellowing, odor, and molecular weight loss of polybutylene adipate terephthalate resin due to polymer decomposition and degradation in the heat treatment step. Further, productivity can be also improved.

The molded body solidified by cooling in the water tank is preferably kept under given temperature in the range of 20°C to 50°C for 1 minute or more (preferably 10 minute or more, more preferably 30 minute or more) before heat treatment. In heat treatment, the thickness of the molded body may change in some cases due to its own weight, however, the change in thickness of the molded body can be reduced by keeping the molded body in the range of 20°C to 50°C after solidification by cooling. For example, after solidification by cooling in a water tank, the molded body may be dried with a continuous dryer which has a first area of a hot air oven to keep the molded body at relative low temperature and a subsequent area of the hot air oven to heat treatment the molded body at relative high temperature.

In order to impart desired functions, the three-dimensional network structure may contain the above various additives. These additives may be included in any step out of steps from a manufacturing step for the thermoplastic resin to a molding step for the three-dimensional network structure, or a polybutylene adipate terephthalate resin containing the additives in advance may be used. The various additives are preferably kneaded into the resin at the time of melt-extrusion to adjust the additive contents according to the color tone or the appearance quality after the resin is melted.

The manufacturing method for the three-dimensional network structure of the present invention is not limited to the above manufacturing method, and the three-dimensional network structure of the present invention may be manufactured by, for example, stacking a network structure made of the hollow fiber, a network structure in which the solid fiber and the hollow fiber coexist, and a network structure made of the solid fiber in this order and integrating these network structures through adhesion.

### <Nozzle>

Hereinafter, a multi-row nozzle having a plurality of orifices having a plurality of different orifice hole diameters will be specifically described.

In order to obtain the three-dimensional network structure of the present invention, a nozzle shape, a nozzle cross section, nozzle hole arrangement, and the like are preferably set to be optimum. Regarding the nozzle shape, the diameters of orifices for forming thin fibers are preferably 1.5 mm or less, and the diameters of orifices for forming thick fibers are preferably 2.0 mm or more. Also, the nozzle orifices for forming thick fibers preferably have hollow-forming shapes, and examples of nozzles with such shapes include C-type nozzles, nozzles having triple-bridge shapes, and the like. Among these nozzles, nozzles having triple-bridge shapes are preferable from the viewpoint of resistance to pressure. An inter-hole pitch of the orifices for forming thin fibers and an inter-hole pitch of the orifices for forming thick fibers are each preferably 4 mm or more and 12 mm or less and further preferably 5 mm or more and 11 mm or less. Examples of the nozzle hole arrangement include lattice arrangement, circumferential arrangement, staggered arrangement, and the like, and lattice arrangement or staggered arrangement is preferable from the viewpoint of the appearance quality of the network structure. Here, each of the inter-hole pitches is the distance between the centers of the nozzle holes, and there are: an inter-hole pitch in the width direction of a three-dimensional network structure to be obtained (hereinafter, referred to as "width-direction inter-hole pitch"); and an inter-hole pitch in the thickness direction of a three-dimensional network structure to be obtained (hereinafter, referred to as "thickness-direction inter-hole pitch"). Both the width-direction inter-hole pitch and the thickness-direction inter-hole pitch are preferably within the above range.

Examples of a nozzle for obtaining the three-dimensional network structure including the coexistence region include a nozzle composed of the following three groups (a group "a", a coexistence group "ab", and a group "b"). The group "b", the coexistence group "ab", and the group "a" are preferably disposed in this order from the upper side to the lower side in the thickness direction (height direction) of a nozzle arrangement region.
Group "a": An orifice hole group composed of orifice holes for solid fibers which are arranged in a plurality of rows in the thickness direction
Coexistence group "ab": An orifice hole group composed of the orifice holes for solid fibers and orifice holes for hollow fibers which are arranged in a coexisting manner in a plurality of rows in the thickness direction
Group "b": An orifice hole group composed of the orifice holes for hollow fibers which are arranged in a plurality of rows in the thickness direction

Examples of another nozzle for obtaining the three-dimensional network structure including the coexistence region include a nozzle composed of the following two groups (a group α and a group β).
Group α: An orifice hole group composed of the orifice holes for solid fibers which are arranged in a plurality of rows in the thickness direction
Group β: An orifice hole group composed of the orifice holes for hollow fibers which are arranged in a plurality of rows in the thickness direction

From the viewpoint of enabling simplification of the configuration of the nozzle, the above nozzle composed of the group α and the group β is more preferable, and it is preferable that the upper half and the lower half of the nozzle arrangement region in the thickness direction (height direction) are respectively the group β and the group α. Although the number of the orifice hole groups of the nozzle is two, fibers spun from near the boundary surfaces of the group α and the group β form a coexistence region in which solid fibers and hollow fibers coexist, whereby the network structure of the present invention composed of the three regions in the thickness direction can be obtained.

In order to obtain a three-dimensional network structure in which the difference between the compression durabilities of both respective surfaces thereof is small, the difference between the width-direction inter-hole pitch of the orifices for solid fibers and the width-direction inter-hole pitch of the orifices for hollow fibers is preferably made small. Specifically, the difference is preferably 2 mm or less, more preferably 1 mm or less, and further preferably 0 mm, i.e. the width-direction inter-hole pitches are further preferably equal to each other. Although the reason why the difference between the width-direction inter-hole pitch of the orifices for solid fibers and the width-direction inter-hole pitch of the orifices for hollow fibers being small leads to a small difference between the compression durabilities of both respective surfaces is not completely obvious, the reason is inferred to be as follows. Hereinafter, the difference between the width-direction inter-hole pitch of the orifices for solid fibers and the width-direction inter-hole pitch of the orifices for hollow fibers is simply referred to as "the difference between the width-direction inter-hole pitches".

The difference between the width-direction inter-hole pitches being small in the coexistence region in which solid fibers and hollow fibers coexist means that the numbers of the solid fibers and the hollow fibers as constituents in the coexistence region are approximate to each other. When the numbers of the solid fibers and the hollow fibers as constituents are approximate to each other, the solid fibers have, fiber by fiber, a plurality of contact points with the hollow fibers, and the hollow fibers have, fiber by fiber, a plurality of contact points with the solid fibers. Therefore, it is considered that, regardless of from which out of both surfaces pressure is applied, stress easily propagates so that the difference between the compression durabilities of both respective surfaces becomes small.

Meanwhile, a case where a network structure is formed with a nozzle in which the difference between the width-direction inter-hole pitches is large is as follows. In the coexistence region in which solid fibers and hollow fibers coexist, for example, when the number of the solid fibers as constituents is larger than the number of the hollow fibers as constituents, some of the solid fibers have almost no contact points with the hollow fibers in the coexistence region. Consequently, it is considered that, when pressure is applied from the side on which the surface mainly composed of the solid fibers is present, these solid fibers having almost no contact points with the hollow fibers cannot sufficiently propagate stress to the hollow fibers. Also, it is considered that, when pressure is applied from the side on which the surface mainly composed of the hollow fibers is present, the hollow fibers cannot sufficiently propagate stress to these solid fibers having almost no contact points with the hollow fibers.

That is, in a case where a three-dimensional network structure is formed with a nozzle in which the difference between the width-direction inter-hole pitches is large, the direction of stress propagation is divided into the thickness direction and a direction orthogonal to the thickness direction so that the efficiency of stress propagation decreases in the coexistence region in which the solid fibers and the hollow fibers coexist. As a result, it is considered that the difference between the compression durability obtained upon pressure application from the solid fiber side and the compression durability obtained upon pressure application from the hollow fiber side becomes large.

The present application claims benefit of priority to Japanese Patent Application No. 2023-168862 filed on September 28, 2023. The entire contents of the specification of Japanese Patent Application No. 2023-168862 filed on September 28, 2023 are incorporated herein by reference.

### EXAMPLES

Hereinafter, the present invention will be specifically described with Examples. However, the scope of the present invention is not limited by the following Examples. The present invention can be carried out with modifications within a range conforming to the gist described above and/or below, and all of which are included in the technical scope of the present invention.

The characteristic values of the three-dimensional network structure in Examples 1 to 4 and Comparative Examples 1 to 2 were measured by the following methods. The sample size described below was the standard size for the measurement, however, a sample in available size was alternatively used in case of insufficiency in sample size.

### (1) Average Fiber Diameter

Each of the three-dimensional network structures was cut into a size of 10 cm×10 cm in longitudinal and lateral directions, and a continuous filament having a hollow cross section and having a length of about 5 mm was collected from each of 10 portions. Then, an optical microscope was used to focus on portions for measuring fiber diameters of the respective continuous filaments having been collected and to measure the fiber diameters, and an average value (n=10) of the fiber diameters of the hollow cross sections at the 10 respective portions was obtained. In addition, an average value of fiber diameters of solid cross sections was also obtained in the same manner as the average value of the fiber diameters of the hollow cross sections.

### (2) Degree of Hollowness

10 continuous filaments were randomly taken out from each of the three-dimensional network structures. Then, the continuous filaments were cut into round slices, the round slices were placed on a glass slide in a state of being raised in the fiber axial direction, and the fiber cross sections taken in the direction in which the round slices were cut were observed with an optical microscope. At this time, only continuous filaments having hollow cross sections as fiber cross sections thereof were selected, an area (a) within the outer circumferential line of each of the fibers and an area (b) of the hollow portion of the fiber were calculated, a degree of hollowness was calculated based on the following formula, and an average value (n=10) of the degrees of hollowness of the selected continuous filaments having hollow cross sections was obtained. $Degree of hollowness \left(%\right) = \left(b\right) / \left(a\right) \times 100$

### (3) Thickness and Apparent Density

Each of the three-dimensional network structures was cut into a size of 10 cm×10 cm in the longitudinal and lateral directions, and the obtained sample was left at rest for 24 hours under no load. Thereafter, a test piece thickness meter (model "FD-80N" manufactured by KOBUNSHI KEIKI CO., LTD.) was used to measure the height at one location which was the center of the sample, and this height of the sample was regarded as a thickness of the three-dimensional network structure. Furthermore, the sample was placed on an electronic balance, and the weight of the sample was measured. The height of the sample was multiplied by the area (100 cm²) defined by the longitudinal and lateral sides of the sample to obtain a volume of the sample, and the weight of the sample was divided by the volume to obtain an apparent density. The aforementioned operation was performed three times, and average values (n=3) of the thicknesses and the apparent densities of the three-dimensional network structure were obtained.

### (4) Apparent Densities of One Surface and Other Surface

Each of the three-dimensional network structures was cut into a size of 5 cm×5 cm in the longitudinal and lateral directions, and a thickness (t1) and a weight (w1) of the obtained sample were measured in the same manner as in (3). Thereafter, the sample was cut such that the resultant cross section became perpendicular to the thickness direction and the sample was divided into two equal pieces in the thickness direction. A thickness (t2) and a weight (w2) of a sample mainly composed of hollow fibers were measured, and the weight (w2 (g)) was divided by a volume (5×5×t2 (cm³)) to calculate an apparent density (g/cm³) of the sample mainly composed of hollow fibers. This apparent density (g/cm³) was regarded as an apparent density of one surface. Then, a value resulting from subtracting the weight (w2 (g)) from the weight (w1 (g)) was divided by a volume (5×5×(t1-t2) (cm³)) to calculate an apparent density (g/cm³) of a sample mainly composed of solid fibers. This apparent density (g/cm³) was regarded as an apparent density of the other surface. Each of these apparent densities was an average value (n=3).

### (5) Molar Ratio of Terephthalic Acid Unit to Adipic Acid Unit of Polybutylene Adipate Terephthalate Resin

The molar ratio of the terephthalic acid unit to the adipic acid unit of each of polybutylene adipate terephthalate resins was measured through ¹H-NMR at a resonance frequency of 600 MHz. The NMR device AVANCE-NEO 600 manufactured by Bruker Corporation was used as a measurement device, and measurement was performed as follows.

10 to 15 mg of a sample was dissolved in a solvent in which the volume ratio of deuterated chloroform to trifluoroacetic acid was 85/15. Then, an NMR tube was filled with the resultant solution, and measurement was performed. Deuterated chloroform was used as a lock solvent, the standby time was set to 1 second, the data acquisition time was set to 4 seconds, and the number of times of integration was set to 64 times.

When the peak of chloroform is set to 7.28 ppm, the peak of adipic acid is detected at 2.45 ppm, and the peak of terephthalic acid is detected at 8.15 ppm.

When the peak integral value of adipic acid is represented by A and the peak integral value of terephthalic acid is represented by B, the molar ratio of the terephthalic acid unit to the adipic acid unit of the polybutylene adipate terephthalate resin can be expressed by the following formula. $Molar ratio = \left(\left(B/4\right)/\left(A/4\right)\right)$

### (6) Melting Point (Tm)

A sample was collected from the three-dimensional network structure and weighed out such that the mass of the sample was 2.0 mg ± 0.1 mg. Then, measurement was performed by using a differential scanning calorimeter (Discovery DSC25 manufactured by TA Instruments Corporation) under a condition of a nitrogen atmosphere at a temperature increase rate of 20°C/min, to obtain a DSC curve. From the DSC curve, a temperature in an endothermic peak (melting peak) was obtained. The above operation was performed 3 times, and the average value of the melting points was obtained (n=3).

### (7) Enthalpy of fusion

A sample was collected from each of the three-dimensional network structures and weighed out such that the mass of the sample was 2.0 mg ± 0.1 mg. Then, measurement was performed by using the differential scanning calorimeter (Discovery DSC25 manufactured by TA Instruments Corporation) under a condition of a nitrogen atmosphere at a temperature increase rate of 20°C/min, to obtain a DSC curve. From the DSC curve, an integral value of an endothermic peak (melting peak) was obtained, thereby evaluating an enthalpy of fusion (J/g).

The integral value of the endothermic peak (melting peak) was obtained as follows. That is, a point at which a curve related to the endothermic peak (melting peak) started to be away from the low-temperature side of a baseline was defined as a start point, a point at which the curve started to be in contact with the high-temperature side of the baseline was defined as an end point, a straight line connecting the start point and the end point was drawn, and a region enclosed by the straight line and the curve was integrated to obtain the enthalpy of fusion. The above operation was performed 3 times, and the average value of the melting enthalpies was obtained (n=3). The above start point was regarded as a melting-start onset temperature (°C).

### (8) Low-temperature Phase Enthalpy

In the DSC curve in the above item (7), an enthalpy of an endothermic peak in which the DSC curve had a minimum value in the range from 30°C to 70°C was obtained, and this enthalpy was defined as a low-temperature phase enthalpy. An integral value of the endothermic peak in the low-temperature phase region was obtained as follows. That is, a point at which a curve related to the endothermic peak started to be away from the low-temperature side of a baseline was defined as a start point, a point at which the curve started to be in contact with the high-temperature side of the baseline was defined as an end point, a straight line connecting the start point and the end point was drawn, and a region enclosed by the straight line and the curve in the range from 30°C to 70°C was integrated to obtain the low-temperature phase enthalpy. The above operation was performed 3 times, and the average value of the low-temperature phase enthalpies was obtained (n=3). The above start point was regarded as a low-temperature phase onset temperature (°C). An example of the experiment data is shown in FIG. 1.

### (9) Melt Flow Rate (MFR)

The polybutylene adipate terephthalate resin was dried in a vacuum at 80°C for 2 hours or more. Then, a melt flow rate (MFR) was quickly measured such that absorption of water in air was prevented as much as possible. The melt flow measurement was performed according to ISO 1133 by using the Melt Indexer F-F01 manufactured by Toyo Seiki Seisaku-sho, Ltd. The measurement temperature was set to 190°C, and the load was set to 2.16 kg. The above operation was performed 3 times, and the average value of the melt flow rates was obtained (n=3).

### (10) 40°C-compression residual strain

Each of the three-dimensional network structures was cut into a size of 10 cm×10 cm. Then, a pre-processing thickness (c) of the obtained sample was measured through the method described in the above (3). The sample, the thickness of which was measured, was sandwiched between jigs capable of holding the sample in a 50%-compressed state, was put into a dryer controlled to be at 40°C, and was left at rest for 22 hours. Thereafter, the sample was taken out, was cooled to eliminate compressive strain, and was left at rest for 30 minutes. Then, a thickness (d) of the sample was measured through the method described in the above (3). These thicknesses were inputted to the following formula to obtain a 40°C-compression residual strain. The aforementioned operation was performed three times, and an average value (n=3) of the 40°C-compression residual strains was obtained. $40 ° C - compression residual strain \left(%\right) = \left(\left(c\right)-\left(d\right)\right) / \left(c\right) \times 100$

### (11) Post-Repeated-Compression Residual Strain

Each of the three-dimensional network structures was cut into a size of 10 cm×10 cm. Then, a pre-compression thickness (e) of the obtained sample was measured through the method described in the above (3). Immediately thereafter, the sample, the thickness of which was measured, was subjected to repeated compression from the one surface (high-density surface) side under the following conditions by using a constant-load-type repeated compression tester (STM-536 manufactured by KOBUNSHI KEIKI CO., LTD.). As a pressure applicator, a circular flat-lower-surface pressure applicator that had a bottom surface with an edge portion having a curvature radius of 25±1 mm and that had a diameter of 250±1 mm and a thickness of 3 mm was used. The load was set to 750 N±20 N, the frequency of compression was set to 70±5 times per minute, and the number of times of repeated compression was set to 13,000 times. After the repeated compression was ended, the sample was left at rest for 10±0.5 minutes in a state where no force was applied. Thereafter, a post-repeated-compression thickness (f) was measured through the method described in the above (3). These thicknesses were inputted to the following formula to obtain a post-repeated-compression residual strain. The aforementioned operation was performed three times, and an average value (n=3) of the residual strains after the repeated compression was performed from the one surface side was obtained.$Post - repeated - compression residual strain \left(%\right) = \left(\left(e\right)-\left(f\right)\right) / \left(e\right) \times 100$

In addition, a residual strain after the repeated compression was performed from the other surface (low-density surface) side was obtained through the method identical to the above method, except that a separate sample was prepared and was subjected to the repeated compression from the other surface side of the sample.

Lastly, the residual strain after the repeated compression was performed from the one surface side was defined as R₁, the residual strain after the repeated compression was performed from the other surface side was defined as R₂, and the absolute value of the difference between the value of the R₁ and the value of the R₂ was obtained.

### (12) 25%-Compression Hardness

Each of the three-dimensional network structures was cut into a size of 10 cm×10 cm, and the obtained sample was left at rest for 24 hours under no load in an environment of 23°C±2°C. Then, measurement was performed in an environment of 23°C±2°C according to the method in ISO 2439 (2008) E by using AUTOGRAPH AG-X plus manufactured by Shimadzu Corporation. Specifically, a pressure application plate having a diameter (φ) of 50 mm was disposed at the center position on the one surface (high-density surface) side of the sample, and a thickness at which the load became 0.5 N was measured. This thickness was regarded as an initial thickness. With the position of the pressure application plate at this time being defined as a zero point, preliminary compression to 75% of the initial thickness was performed at a speed of 100 mm/min one time, and the pressure application plate was returned to the zero point at the same speed. Then, the sample was left at rest for 4 minutes in this state. Immediately thereafter, compression to a thickness that was 75% of the initial thickness was performed at a speed of 100 mm/min, and the load at this time was measured. This load was regarded as a 25%-compression hardness (N/φ50 mm) obtained upon pressure application from the one surface side. The aforementioned operation was performed three times, and an average value (n=3) of the 25%-compression hardnesses obtained upon pressure application from the one surface side was obtained.

In addition, a 25%-compression hardness obtained upon pressure application from the other surface (low-density surface) side was obtained through the method identical to the above method, except that the pressure application plate having a diameter (φ) of 50 mm was disposed at the center position on the other surface side of a sample. For performing measurement of the compression hardness obtained upon pressure application from the one surface side and the compression hardness obtained upon pressure application from the other surface side, respective different samples were prepared, and the same applies to the following (13) and subsequent measurements.

Lastly, a larger value and a smaller value out of the 25%-compression hardness obtained upon pressure application from the one surface side and the 25%-compression hardness obtained upon pressure application from the other surface side were respectively defined as H₁ and H₂, and the value of H₁/H₂ was calculated.

### (13) 40%-Compression Hardness

A 40%-compression hardness obtained upon pressure application from the one surface side was obtained through the method described in the above (12), except that, immediately after the sample was left at rest for 4 minutes, compression to a thickness that was 60% of the initial thickness was performed at a speed of 100 mm/min, and the load at this time was measured and was regarded as a 40%-compression hardness (N/φ50 mm) obtained upon pressure application from the one surface side.

In addition, a 40%-compression hardness obtained upon pressure application from the other surface (low-density surface) side was obtained through the same method as that for the 40%-compression hardness obtained upon pressure application from the one surface side, except that the pressure application plate having a diameter (φ) of 50 mm was disposed at the center position on the other surface side of a sample.

Lastly, a larger value and a smaller value out of the 40%-compression hardness obtained upon pressure application from the one surface side and the 40%-compression hardness obtained upon pressure application from the other surface side were respectively defined as H₃ and H₄, and the value of H₃/H₄ was calculated.

### (14) Compressive Deflection Coefficient

A 65%-compression hardness obtained upon pressure application from the one surface side was obtained through the method described in the above (12), except that, immediately after the sample was left at rest for 4 minutes, compression to a thickness that was 35% of the initial thickness was performed at a speed of 100 mm/min, and the load at this time was measured and was regarded as a 65%-compression hardness (N/φ50 mm) obtained upon pressure application from the one surface side.

In addition, a 65%-compression hardness obtained upon pressure application from the other surface (low-density surface) side was obtained through the same method as that for the 65%-compression hardness obtained upon pressure application from the one surface side, except that the pressure application plate having a diameter (φ) of 50 mm was disposed at the center position on the other surface side of a sample.

A value resulting from dividing the value of the 65%-compression hardness obtained upon pressure application from the one surface side by the value of the 25%-compression hardness obtained upon pressure application from the one surface side was regarded as a compressive deflection coefficient obtained upon pressure application from the one surface side. The aforementioned operation was performed three times, and an average value (n=3) of the compressive deflection coefficients obtained upon pressure application from the one surface side was obtained. In addition, a compressive deflection coefficient obtained upon pressure application from the other surface side was also obtained through the same method as that for the compressive deflection coefficient obtained upon pressure application from the one surface side.

Lastly, the absolute value of the difference between the compressive deflection coefficient obtained upon pressure application from the one surface side and the compressive deflection coefficient obtained upon pressure application from the other surface side was obtained.

The polybutylene adipate terephthalate resins were synthesized through the following methods.

### <Resin A>

In a reaction tank equipped with a stirrer, a thermometer, and a distillation cooler, 1,4-butanediol, adipic acid, and dimethyl terephthalate were mixed in proportions of 1.5 moles, 0.4 moles, and 0.6 moles, respectively. Then, the resultant mixture was fed with 300 ppm of tetrabutyl titanate (manufactured by Sigma-Aldrich Co., LLC.) as a titanium-based catalyst. Thereafter, a transesterification reaction and an esterification reaction were performed for 2 hours under a normal pressure and at 220°C, to prepare a prepolymer. The prepolymer was heated to 240°C, and then subjected to a polycondensation reaction at 0.1 mmHg for 2 hours. The obtained resin A was cooled, and then cut by using a pellet cutter, to produce pellets.

### <Resin B>

A resin B was produced in the same method as that for the resin A except that, unlike in the production of the resin A, the amounts of the adipic acid and the dimethyl terephthalate were changed to 0.53 moles and 0.47 moles, respectively. The obtained resin B was cooled, and then cut by using a pellet cutter, to produce pellets.

### [Example 1]

The resin A was used as a raw material and was extruded as molten resin downward of the nozzle at a spinning temperature of 240°C, at a single-hole extrusion rate from each hollow hole of 1.2 g/min, and at a single-hole extrusion rate from each solid hole of 0.84 g/min. A nozzle effective surface having a length in the width direction of 96 mm and a length in the thickness direction of 31 mm had an upper half in the thickness direction (height direction) and a lower half in the thickness direction. The upper half was provided with a portion obtained by arranging orifices in a staggered pattern with the width-direction inter-hole pitch being 6 mm and with the thickness-direction inter-hole pitch being 5.2 mm, each of the orifices having a triple-bridge hollow-forming cross section with the outer diameter being 3.0 mm and with the inner diameter being 2.6 mm. The lower half was provided with a portion obtained by arranging orifices in a staggered pattern with the width-direction inter-hole pitch being 6 mm and with the thickness-direction inter-hole pitch being 5.2 mm, each of the orifices having a solid cross section with the outer diameter being 1.0 mm.

A water tank was disposed such that the surface of cooling water therein was located 30 cm below the nozzle surface of the nozzle for extruding molten resin. The temperature of the water was set to 12°C. A pair of take-up conveyors were disposed in the water tank so as to be partially exposed from the surface of the water. Each of the take-up conveyors had an endless net made of stainless steel and having a width of 20 cm and was disposed such that the width direction of the nozzle surface and the conveyor were parallel to each other. The opening width of the endless net was set to 30 mm. In order to form side surface portions, aluminum plates were each disposed at an angle of 90 degrees relative to the direction of the net, and water was caused to flow at a speed of 1.0 L/min, thereby forming side surface portions.

The above molten resin was linearly extruded to an opening portion of the net of the above conveyor, onto the net of the above conveyor, and to the aluminum plates as the above side surface portions, and the resultant continuous filament was caused to flow downward so as to be curved and twisted, whereby loops were formed. Thus, while contact portions were fused together, a three-dimensional network configuration was formed. While both surfaces of the three-dimensional network configuration in the molten state were sandwiched between the take-up conveyors, the structure was drawn into the cooling water at a speed of 0.86 m/min so as to be solidified. Consequently, both surfaces in the thickness direction and both surfaces in the side surface direction were flattened. Then, the structure was cut into a predetermined size and was left at rest in a space at 25°C for 1 hour. Thereafter, heating was performed with hot air at 90°C for 20 minutes, whereby a three-dimensional network structure having a width of 100 mm was obtained.

### [Example 2]

A three-dimensional network structure was obtained in the same manner as in Example 1, except that: the single-hole extrusion rate from each hollow hole was set to 1.8 g/min; the single-hole extrusion rate from each solid hole was set to 1.20 g/min; and the take-up speed was set to 1.43 m/min.

### [Example 3]

A three-dimensional network structure was obtained in the same manner as in Example 1, except that: the single-hole extrusion rate from each hollow hole was set to 1.8 g/min; the single-hole extrusion rate from each solid hole was set to 1.20 g/min; the distance from the nozzle surface to the surface of the cooling water in the water tank was set to 40 cm; and the take-up speed was set to 1.43 m/min.

### [Example 4]

A three-dimensional network structure was obtained in the same manner as in Example 1, except that: an adduct obtained by adding 0.1% by mass of water with respect to 100% by mass of a solid component of the resin A as a raw material was used instead of the resin A; the distance from the nozzle surface to the surface of the cooling water in the water tank was set to 18 cm; and the take-up speed was set to 0.95 m/min.

### [Comparative Example 1]

A three-dimensional network structure was obtained in the same manner as in Example 1, except for the following differences. A nozzle having a nozzle effective surface that had a length in the width direction of 96 mm and a length in the thickness direction of 31 mm and in which two portions were formed was used. One of the portions was obtained by arranging orifices in a staggered pattern with the width-direction inter-hole pitch being 10 mm and with the thickness-direction inter-hole pitch being 7.5 mm, each of the orifices having a triple-bridge hollow-forming cross section with the outer diameter being 3.0 mm and with the inner diameter being 2.6 mm. The other one of the portions was obtained by arranging orifices in a staggered pattern with the width-direction inter-hole pitch being 2.5 mm and with the thickness-direction inter-hole pitch being 3.7 mm, each of the orifices having a solid cross section with the outer diameter being 0.7 mm. In addition, the single-hole extrusion rate from each hollow hole was set to 2.0 g/min, the single-hole extrusion rate from each solid hole was set to 0.50 g/min, the distance from the nozzle surface to the surface of the cooling water in the water tank was set to 18 cm, and the take-up speed was set to 1.14 m/min.

### [Comparative Example 2]

A three-dimensional network structure was obtained in the same manner as in Example 1, except that: the resin B was used as a raw material; the spinning temperature was set to 190°C; the distance from the nozzle surface to the surface of the cooling water in the water tank was set to 28 cm; and the take-up speed was set to 0.95 m/min.

Table 1 shows production conditions and the characteristics of the obtained three-dimensional network structure in Examples from 1 to 4 and Comparative Examples from 1 to 2. In Table 1, the characteristic value is the average of the value by operations of multiple times.

**[Table 1]**

| | | | Example 1 | Example 2 | Example 3 | Example 4 | Comparative Example 1 | Comparative Example 2 |
|---|---|---|---|---|---|---|---|---|
| Manufacturing conditions | Spinning temperature: °C | | 240 | 240 | 240 | 240 | 240 | 190 |
| | Single-hole extrusion rate | Hollow hole: g/min | 1.2 | 1.8 | 1.8 | 1.2 | 2.0 | 1.2 |
| | | Solid hole: g/min | 0.84 | 1.20 | 1.20 | 0.84 | 0.50 | 0.84 |
| | Distance (from nozzle surface to surface of cooling water in water tank): cm | | 30 | 30 | 40 | 18 | 18 | 28 |
| | Take-up speed: m/min | | 0.86 | 1.43 | 1.43 | 0.95 | 1.14 | 0.95 |
| Resin | Type of resin | | A | A | A | A | A | B |
| | Resin melting point: °C | | 150 | 150 | 150 | 150 | 150 | 120 |
| | Melt flow rate: g/10 min | | 6.5 | 6.5 | 6.5 | 13.9 | 6.5 | 20 |
| | PBAT content: % by mass | | 100 | 100 | 100 | 100 | 100 | 100 |
| | Molar ratio (terephthalic acid unit/adipic acid unit) | | 1.5 | 1.5 | 1.5 | 1.5 | 1.5 | 0.89 |
| Three-dimensional network structure | Average fiber diameter | Hollow fiber: mm | 0.69 | 0.83 | 0.65 | 0.64 | 0.82 | 0.47 |
| | | Solid fiber: mm | 0.48 | 0.53 | 0.44 | 0.48 | 0.35 | 0.36 |
| | | Difference in average fiber diameter between both fibers: mm | 0.21 | 0.30 | 0.21 | 0.16 | 0.47 | 0.11 |
| | Degree of hollowness of hollow fiber: % | | 18.8 | 24.2 | 21.9 | 6.0 | 21.2 | 5.5 |
| | Apparent density | Entire three-dimensional network structure: g/cm³ | 0.052 | 0.051 | 0.052 | 0.049 | 0.051 | 0.048 |
| | | One (high-density-side) surface: g/cm³ | 0.084 | 0.064 | 0.088 | 0.072 | 0.059 | 0.068 |
| | | Other (low-density-side) surface: g/cm³ | 0.039 | 0.043 | 0.035 | 0.039 | 0.048 | 0.039 |
| | | Difference between both surfaces: g/cm³ | 0.045 | 0.021 | 0.053 | 0.033 | 0.011 | 0.029 |
| | Thickness: mm | | 28.5 | 26.6 | 25.9 | 28.5 | 27.7 | 24.3 |
| | Melting-start onset temperature: °C | | 94.8 | 94.6 | 95.1 | 99.5 | 99.8 | 95.1 |
| | Enthalpy of fusion: J/g | | 26.4 | 22.3 | 21.8 | 27.1 | 26.4 | 17.8 |
| | Low-temperature phase onset temperature: °C | | 35.7 | 35.4 | 35.4 | 37.2 | 37.5 | 33.6 |
| | Low-temperature phase enthalpy: J/g | | 0.79 | 1.04 | 1.30 | 1.40 | 1.02 | 2.72 |
| | 40°C-compression residual strain: % | | 10.7 | 14.1 | 13.9 | 13.0 | 13.3 | 17.9 |
| | Post-repeated-compression residual strain | One (high-density-side) surface: % | 7.1 | 9.0 | 9.2 | 11.2 | 8.9 | 10.8 |
| | | Other (low-density-side) surface: % | 7.6 | 9.3 | 7.7 | 12.2 | 19.3 | 11.0 |
| | | Difference between both surfaces: % | 0.5 | 0.3 | 1.5 | 1.0 | 10.4 | 1.6 |
| | 25%-compression hardness | One (high-density-side) surface: N/Φ50 | 17.3 | 17.5 | 12.8 | 16.9 | 12.8 | 7.9 |
| | | Other (low-density-side) surface: N/Φ50 | 15.0 | 13.4 | 11.0 | 13.5 | 11.0 | 7.1 |
| | | Ratio between both surfaces: - | 1.15 | 1.31 | 1.16 | 1.25 | 1.16 | 1.11 |
| | 40%-compression hardness | One (high-density-side) surface: N/Φ50 | 26.7 | 26.4 | 23.5 | 23.8 | 23.5 | 16.2 |
| | | Other (low-density-side) surface: N/Φ50 | 24.4 | 21.1 | 21.2 | 21.7 | 21.2 | 14.3 |
| | | Ratio between both surfaces: - | 1.09 | 1.25 | 1.11 | 1.10 | 1.11 | 1.13 |
| | Compressive deflection coefficient | One (high-density-side) surface: - | 3.30 | 3.43 | 4.19 | 2.79 | 4.19 | 3.16 |
| | | Other (low-density-side) surface: - | 3.79 | 4.46 | 4.39 | 3.77 | 4.39 | 4.08 |
| | | Difference between both surfaces: - | 0.49 | 1.03 | 0.20 | 0.98 | 0.20 | 0.92 |

Each of the three-dimensional network structures in Exmaples 1 to 4 exhibited excellent compression recoverability after compression at the usage environment temperature and had excellent compression durabilities on both respective surfaces thereof, with the difference between the compression durabilities of both respective surfaces being small.

## Claims

1. A three-dimensional network structure having a three-dimensional random loop-bonded configuration and comprising a continuous filament made from a thermoplastic resin composition, wherein
the thermoplastic resin composition contains 70% by mass or more of a polybutylene adipate terephthalate resin,
an apparent density of one surface of the three-dimensional network structure is higher than an apparent density of the other surface of the three-dimensional network structure,
a residual strain R₁ after compression is repeatedly performed 13,000 times at a load of 750 N from the one surface side and a residual strain R₂ after compression is repeatedly performed 13,000 times at a load of 750 N from the other surface side are each 20% or less,
an absolute value of a difference between a value of the R₁ and a value of the R₂ is 10% or less, and
the three-dimensional network structure has a 40°C-compression residual strain of 15% or less.

2. The three-dimensional network structure according to claim 1, wherein
the polybutylene adipate terephthalate resin contains an adipic acid unit and a terephthalic acid unit, and
a molar ratio of the terephthalic acid unit to the adipic acid unit is 1.0 or more and 3.0 or less.

3. The three-dimensional network structure according to claim 1, wherein the polybutylene adipate terephthalate resin has a melting point of 125°C or more and 180°C or less.

4. The three-dimensional network structure according to claim 1, wherein the three-dimensional network structure has an apparent density of 0.005 g/cm³ or more and 0.20 g/cm³ or less.

5. The three-dimensional network structure according to claim 1, wherein, in a case where a larger value and a smaller value out of a 25%-compression hardness obtained upon pressure application from the one surface side and a 25%-compression hardness obtained upon pressure application from the other surface side are respectively defined as H₁ and H₂, H₁/H₂ is 1.03 or more.

6. The three-dimensional network structure according to claim 1, wherein, in a case where a larger value and a smaller value out of a 40%-compression hardness obtained upon pressure application from the one surface side and a 40%-compression hardness obtained upon pressure application from the other surface side are respectively defined as H₃ and H₄, H₃/H₄ is 1.05 or more.

7. The three-dimensional network structure according to claim 1, wherein an absolute value of a difference between a compressive deflection coefficient obtained upon pressure application from the one surface side and a compressive deflection coefficient obtained upon pressure application from the other surface side is 5.0 or less.

8. The three-dimensional network structure according to claim 1, wherein an enthalpy of an endothermic peak in which a differential scanning calorimetry curve regarding the continuous filament measured by using a differential scanning calorimeter has a minimum value in a range from 30°C to 70°C, is 2.5 J/g or less.

9. The three-dimensional network structure according to claim 1, wherein an absolute value of a difference between the apparent density of the one surface and the apparent density of the other surface is 0.015 g/cm³ or more.

10. A cushioning material comprising the three-dimensional network structure according to any one of claims 1 to 9, wherein the cushioning material is reversibly usable.
